

June 18, 1935.

S. H. COHEN ET AL

2,005,221

MULTI-PLY FLASHING STRUCTURE

Filed Jan. 22, 1935



Inventors  
Samuel H. Cohen  
Jacob Wasserman  
by Knight, Brown, Quincy, Tracy  
Atty's

## UNITED STATES PATENT OFFICE

2,005,221

## MULTI-PLY FLASHING STRUCTURE

Samuel H. Cohen, Boston, and Jacob Wasserman,  
Cambridge, Mass.

Application January 22, 1935, Serial No. 2,914

6 Claims. (Cl. 72—127)

This invention relates to flashing structures such, for example, as are embedded in the mortar seams of the side walls of a building to prevent rain water from seeping through the walls and thus impairing them, the ceilings and floors, or other parts of the building. It deals more particularly with a multi-ply or composite flashing structure such as is designed to be placed in a mortar seam and be locked or embedded there-in with sufficient tenacity to resist shifting forces or dislodgment while avoiding as much as possible weakening of the seam.

In accordance with the present invention, we provide a multi-ply flashing structure comprising at least three plies, the inner ply of which is substantially impermeable, non-corrodible sheet metal, such as copper, and the outer ones of which are waterproofed fibrous sheet material bonded facially to the surfaces of the inner ply and presenting in their fibrous texture a multiplicity of exposed recesses, preferably occurring with substantial regularity therein, into which the mortar of a wall seam may freely enter and then harden to lock or embed the structure with the desired grip or tenacity in the resulting seam. It is thus seen that the inner ply of such a flashing structure affords the desired perfect waterproof barrier, whereas the outer plies maintain the desired integrality of the structure as a whole with the wall of the building in which it is used. The flashing structure of the present invention is further advantageous in that it can be made at low cost, inasmuch as the non-corrodible sheet metal constituting the inner ply may be used at much lower weight or thickness than ordinarily by reason of the fact that the outer plies give additional strength or reinforcement to the sheet metal, protect it from being marred or fractured even when it is so thin as to be comparatively easily cut, torn, bent, or distorted, and lend thereto resistance to deformation when it is preformed and/or fixed in place in a particular configuration or shape.

While not restricted thereto, the present invention may be advantageously embodied in flashing structures whose outer plies comprise either coarsely woven fibrous material or felted fibrous material prepared as on papermaking or textile machines. In the case of coarsely woven fibrous material, which is reticulated at the very start, the fibrous material is waterproofed and bonded to the inner metallic ply while retaining or preserving in large measure in its exposed face its original reticulated or open coarse-mesh texture for the purpose of enmeshing mor-

tar, despite the fact that its component threads are preferably adequately coated or protected with suitable waterproofing or water-repelling material and its inner face is masked by a film or thin coating of waterproofing material which also serves as the medium for bonding it to the inner ply. In the case of felted fibrous material, which initially presents substantially smooth faces, the fibrous material is preferably first waterproofed, as by impregnation with suitable waterproofing material, and is then put through an embossing or other operation that creates therein localized compressed areas recessed or offset inwardly from its surface to be exposed to mortar and in which mortar may be entrapped in sufficient amount to be welded strongly to the mortar of a wall seam. In order that the felt may be readily embossed or indented to present the desired reticulated fibrous texture for the reception of mortar, it is preferable that it be prepared with adequate compressibility, such as is possessed by highly absorptive paper felt, and that it be waterproofed by a material, such as bitumen, that yields or "flows" under pressure.

With the foregoing and other features and objects in view, we shall now describe our invention with reference to the accompanying drawing, wherein,—

Figure 1 is a plan view of a fragment of flashing structure embodying our invention. 30

Figure 2 is a similar view of another form or embodiment of our invention.

Figures 3 and 4 represent sections on the lines 3—3 and 4—4 of Figures 1 and 2, respectively.

Figure 5 is a vertical section through a conventional building wall into which our flashing structures may be advantageously incorporated at various localities. 35

The flashing structure of Figure 3 includes, as shown therein, a substantially impermeable inner ply or membrane 10 to each of whose faces is bonded by a film or thin coating of adhesive 12 a coarsely woven fabric 11. The inner ply 10 consists of thin, non-corrodible sheet metal, preferably copper foil such as is available on the market as electrolytic or electrodeposited copper. The outer plies 11 may be such coarsely woven fabrics as burlap or gunny cloth which present large openings or meshes of substantial depth. In making the composite flashing structure, the fabric 11 is preferably first treated with waterproofing material in a manner such that substantially all of its yarns acquire a protective or waterproof coating 13 while its openings or meshes 14 are preserved largely open or un- 55

obstructed for the reception of mortar. Thus, the fabric may be sprayed with molten asphalt or water-dispersed asphalt of sufficient fluidity to run freely through the openings or meshes while 5 impregnating the yarns and depositing thereon and on its constituent fibers the desired protective films or coatings. Comparable results may also be had by running the fabric through a bath of molten asphalt or water-dispersed asphalt of the 10 appropriate fluidity. Separate plies of such waterproofed but porous fabric may then be adhesively secured to the faces of the inner ply 10, the faces of such inner ply being preferably first treated with molten asphalt or equivalent water- 15 proof adhesive material constituting the film 12 for bonding the fabric to the inner ply. Inasmuch as electrolytic copper foil, such as is preferably used as the inner ply material, can be purchased in roll or continuous sheet form, it is 20 possible to build up the composite flashing structure of the present invention progressively from such continuous sheet and from continuous sheets of the waterproofed fabric. For instance, the copper foil may be progressively unwound from a 25 parent roll, be progressively sprayed or otherwise thinly coated substantially uniformly with the molten asphalt, and have progressively placed on each of its coated surfaces a continuous sheet of waterproofed fabric, which may be pressed into 30 the coating while still hot and sticky, as by a pair of rolls, through which the multi-ply sheet may be progressively run. The resulting multi-ply sheet may be cut up into flashing sections of the dimensions desired for use. The coating or film 12 35 thus masks the inner face of the fabric and bonds it throughout to the inner ply 10, but the exposed face of the fabric retains largely its original open coarse-mesh texture and can thus enmesh considerable mortar.

40 The flashing structure of Figure 4 differs from that of Figure 3 essentially in that its outer fibrous plies 15 are made up of felted fibers and in that the recessed or reticulated exposed texture presented thereby results from a separate or special 45 operation. The felt may, as already stated, be produced on papermaking or textile machines and have initially a substantially uniform body thickness distinctly greater than the inner metallic ply 10 of the flashing structure. The felt is rendered 50 weather-resistant, as by impregnation substantially uniformly throughout with asphalt or other suitable waterproofing material. Indeed, the plies 15 may be bituminized felt similar to that sometimes used for roofing and flooring purposes.

55 The impregnated felt may be provided with the desired reticulated surface texture as by an embossing or other operation performed in such a way as to effect marked localized compression of the felt and to create therein a multiplicity of 60 indented areas 16 distributed preferably with substantial regularity thereover and indented or recessed sufficiently from its outer surface to serve as pockets for catching or entrapping a substantial amount of mortar capable of uniting with a 65 layer of mortar distributed over its surface and thus capable of welding the flashing structure in which it appears inseparably to the mortar layer, that is, with such firmness that the flashing structure cannot be dislodged without severe disruption or breakdown of the mortar layer and/or of the flashing structure itself. The indented waterproofed felt plies 15 are bonded, as are the 70 waterproofed woven fabric plies 11, to the inner metallic ply 10 by films or thin coatings 12 of asphalt or other suitable waterproof adhesive.

Flashing structures embodying our invention are useful generally in the walls of buildings. As illustrated in Figure 5, they may be used in a building wall at such regions as 17, where the coping 18 meets the parapet 19; at 20 where the roof beam 21, the parapet 19, and the window superstructure 21 come together; at 22, just above the window frame; at 23, just below the window frame; and at 24, where the spandrel beam 25 and the floor beam 26 join with the wall. In installing the flashing structures of the present invention in any of such localities, it may be desirable to crimp them to zigzag or checker-board configurations or to impart thereto other suitable longitudinal, transverse, or diagonal crimps or bends 15 designed to promote permanent anchorage in the mortar spread over and under their surfaces for forming the seams. It will, of course, be appreciated that mortar is invariably used to effect a bond between the stones that go to make up the 20 wall structure and that mortar seams occurring in building walls in which the flashings of the present invention are employed are maintained intact where they contact with the flashing surfaces, whereas, on the other hand, the mortar 25 seams tend to loosen or weaken when they are interrupted by smooth metallic flashing surfaces.

While it is possible to use various waterproofing materials, such as gums and resins, for the purpose of protecting the fibrous plies of the 30 flashing structures of the present invention against weathering influences, nevertheless, asphalt, pitch, tar, or similar bituminous material is advantageous for such purpose in that it has the desired waterproof, adhesive, and other qualities and is sufficiently inexpensive to make for the desired low cost product. We wish again to observe that by virtue of the comparatively low cost of the fibrous plies used in the multi-ply or composite flashing structures of our invention, it is 40 possible to economize greatly in the amount of copper or other non-corrodible sheet metal put therein and thus to realize an improved article at lowered cost.

We claim:

1. A multi-ply flashing structure adapted to be embedded in a mortar seam and comprising three plies, the inner one being substantially impermeable, non-corrodible sheet metal and the outer ones being waterproofed fibrous sheet material 50 bonded facially to the surfaces of said inner ply and presenting in their fibrous texture a multiplicity of exposed recesses into which the mortar of a seam may enter in substantial amount and harden to lock said structure in such seam. 55

2. A multi-ply flashing structure adapted to be embedded in a mortar seam and comprising three plies, the inner one being substantially impermeable, non-corrodible sheet metal and the outer ones being bituminized fibrous sheet material 60 bonded by said bitumen facially to the surfaces of said inner ply and presenting in their fibrous texture a multiplicity of exposed recesses into which the mortar of a seam may enter in substantial amount and harden to lock said structure in such seam. 65

3. A multi-ply flashing structure adapted to be embedded in a mortar seam and comprising three plies, the inner one being substantially impermeable, non-corrodible sheet metal and the outer ones being waterproofed, coarsely woven fibrous material bonded facially to the surfaces of said inner ply and whose inner faces are masked by a bonding film of waterproofing material but whose exposed faces retain in large measure their origi- 70 75

nal, open coarse-mesh texture to enmesh in substantial amount the mortar of a seam.

4. A multi-ply flashing structure adapted to be embedded in a mortar seam and comprising three plies, the inner one being substantially impermeable, non-corrodible sheet metal and the outer ones being bituminized, coarsely woven fibrous material bonded by said bitumen facially to the surfaces of said inner ply and whose inner faces 10 are masked by a bonding film of said bitumen but whose exposed faces retain in large measure their original, open, coarse-mesh texture to enmesh in substantial amount the mortar of a seam.

5. A multi-ply flashing structure adapted to be 15 embedded in a mortar seam and comprising three plies, the inner one being substantially impermeable, non-corrodible sheet metal and the outer ones being waterproofed felted fibrous material bonded facially to the surfaces of said inner ply,

and presenting on their fibrous texture a multiplicity of exposed localized indentations into which the mortar of a seam may enter in substantial amount and harden to lock said structure in such seam.

6. A multi-ply flashing structure adapted to be embedded in a mortar seam and comprising three plies, the inner one being substantially impermeable, non-corrodible sheet metal and the outer ones being bituminized felted fibrous material 10 bonded facially by said bitumen to the surfaces of said inner ply and presenting in their fibrous texture a multiplicity of exposed localized areas recessed from their outer surfaces into which the mortar of a seam may enter in substantial 15 amount and harden to lock said structure in said seam.

SAMUEL H. COHEN.  
JACOB WASSERMAN.